

[54] METHOD OF REFINING COAL BY CATALYZED SHORT RESIDENCE TIME HYDRODISPROPORTIONATION TO FORM A NOVEL COAL-DERIVED FUEL SYSTEM

[75] Inventors: Lee G. Meyer; Gerald F. Cavaliere, both of Englewood, Colo.

[73] Assignee: Carbon Fuels Corporation, Englewood, Colo.

[21] Appl. No.: 522,933

[22] Filed: May 14, 1990

#### Related U.S. Application Data

[63] Continuation-in-part of Ser. No. 355,528, May 23, 1989, Pat. No. 5,021,148, and a continuation-in-part of Ser. No. 277,603, Nov. 28, 1988, Pat. No. 4,938,782, and a continuation-in-part of Ser. No. 84,270, Aug. 11, 1987, Pat. No. 4,787,915, and a continuation-in-part of Ser. No. 59,288, Jun. 8, 1987, Pat. No. 4,832,831.

[51] Int. Cl. 5 ..... C10G 1/00  
 [52] U.S. Cl. ..... 208/423; 208/431;  
 ..... 208/433; 44/282

[58] Field of Search ..... 208/431, 433, 423;  
 ..... 44/282

[56]

#### References Cited

##### U.S. PATENT DOCUMENTS

4,687,570 8/1987 Sundalam et al. .... 208/431  
 4,842,719 6/1989 MacArthur et al. .... 208/431  
 4,938,782 7/1990 Meyer et al. .... 208/431  
 5,021,148 6/1991 Meyer et al. .... 208/431

Primary Examiner—Jacqueline Howard  
 Attorney, Agent, or Firm—Lee G. Meyer

[57]

#### ABSTRACT

This invention generally relates to a catalyzed short residence time decomposition and volatilization of coal to produce liquid co-products while minimizing production of char and gas without utilization of external hydrogen, that is, hydrogen other than that contained in the coal feedstock. The invention more particularly relates to an improved method of economically producing uniform, fluidic, oil-type transportable fuel systems and fuel compositions and a slate of "value-added" co-products by a catalyzed coal refining process employing short residence time hydrodisproportionation (SRT-HDP). The preferred catalysts are oxides and salts of iron.

24 Claims, 2 Drawing Sheets







**METHOD OF REFINING COAL BY CATALYZED  
SHORT RESIDENCE TIME  
HYDRODISPROPORTIONATION TO FORM A  
NOVEL COAL-DERIVED FUEL SYSTEM**

This application is a continuation-in-part of U.S. patent application Ser. No. 355,528 filed May 23, 1989, now U.S. Pat. No. 5,021,148 issued Jun. 4, 1991 and of its parent, U.S. patent application Ser. No. 277,603 filed Nov. 28, 1988 now U.S. Pat. No. 4,938,782, issued Jul. 3, 1990, and of its parent, U.S. patent application Ser. No. 084,270 filed Aug. 11, 1987 now U.S. Pat. No. 4,787,915 issued Nov. 29, 1988, and of its parent U.S. patent application Ser. No. 059,288 filed Jun. 8, 1987, now U.S. Pat. No. 4,832,831 issued May 23, 1989.

**TECHNICAL FIELD**

These parent, grandparent, great-grandparent, and great-great-grandparent applications, which are incorporated in their entirety by reference as if they were completely set out herein, disclose a coal refining process which economically produces a slate of clean burning value-added products. One process configuration produces non-polluting, fluidic, completely combustible, transportable fuel compositions derived from coal, which compositions contain particulate coal char admixed with liquids obtained from short residence time hydrodisproportionation of coal.

The parent application discloses a partial liquefaction scheme using short residence time hydrodisproportionation to produce petroleum substitutes.

The grandparent application relates to rapid volatilization of the coal particle followed by an uncatalyzed hydrogenation reaction to conserve hydrogen and increase liquid yield.

The great-grandparent application further discloses that the process method can be altered to vary the product and co-product distribution as well as the rheological characteristics of the fuel compositions.

The great-great-grandparent discloses that the method of processing the coal, and specifically hydrodisproportionation, is important in determining both the economics of the process and the slate of value-added co-products.

The ancestor applications, as a whole, relate to volatilization of coal to produce char and liquid co-products without utilization of external hydrogen, i.e., hydrogen other than that contained in the coal feedstock, and more particularly to an improved method of economically producing uniform, fluidic, oil-type transportable fuel systems and fuel compositions and a slate of "value-added" co-products by a coal refining process employing short residence time, high heating rate, hydrogen rearrangement (hydrodisproportionation).

**BACKGROUND ART**

Coal is the world's most abundant fossil fuel. However, coal has three major drawbacks: (1) Coal is a solid and is less easily handled and transported than fluidic or gaseous materials; (2) Coal contains compounds which, on burning, produce the pollutants associated with acid rain; and (3) Coal is not a uniform fuel product, varying in characteristics from region to region and from mine to mine.

In fossil fuels, the ratio of hydrogen atoms to carbon atoms is most important in determining the heating value per unit weight. The higher the hydrogen con-

tent, the more liquid (or gaseous) the fuel, and the greater its heat value. Natural gas, or methane, has a hydrogen-to-carbon ratio of 4 to 1 (this is the maximum); gasoline has a ratio of almost 2.2 to 1; petroleum crude about 2.0 to 1; shale oil about 1.5 to 1; and coal about 1 to 1.

The lignites, peats, and lower calorific value sub-bituminous coals have not had an economic use except in the vicinity of the mine site, for example, mine mouth power generation facilities. This is due primarily to the cost of shipping a lower Btu, higher moisture product as well as to the danger of spontaneous combustion because of the high content of volatile matter which is characteristic of such coals.

The risk of spontaneous combustion of low-rank coals is increased by dehydration, even by non-evaporation methods. Therefore, in order to secure stability of the dehydrated coal in storage and transportation, it has been necessary to cover the coal with an atmosphere of inert gas such as nitrogen or combustion product gas, or to coat it with crude oil so as not to reduce its efficiency as a fuel. However, these methods are not very economical.

Waste coal has somewhat different inherent problems from those of the low-rank coals. Waste coal is sometimes referred to as a "non-compliance coal" because it is too high in sulfur per unit heat value to burn in compliance with the United States Environmental Protection Agency (EPA) standards. Other waste coal is too low in heat value to be transported economically.

The inefficient and expensive handling, transportation and storage of all types of coal (primarily because it is a solid material) prevent coal from being an exportable commodity and cause the conversion of oil-fired systems to coal to be economically unattractive. Liquids are much more easily handled, transported, stored and fired into boilers.

Besides being difficult to transport, coal is a heterogeneous fuel, i.e., coal from different reserves has a wide range of characteristics. Coal from one region (or even of a particular mine) cannot be efficiently combusted in boilers designed for coal from another source. Boilers and pollution control equipment must either be tailored to a specific coal or configured to burn a wide variety of material with a resultant loss in efficiency.

The non-uniformity and transportation problems are compounded by the presence of combustion pollutants in coal such as sulfur and nitrogen compounds which are thought to cause acid rain. The sulfur compounds are of two types: organic and inorganic (pyritic). The fuel bound nitrogen, i.e., organic nitrogen in the coal, combusts to form NO<sub>x</sub>. Further, because of the non-uniformity of coal, it combusts with "hot spots" which result in some of the nitrogen in the combustive air (air is 75% nitrogen by weight) being oxidized to produce NO<sub>x</sub>. This so-called "thermal NO<sub>x</sub>" has heretofore been reduced only by boiler modification systems or expensive catalytic reduction systems.

Raw coal cleaning has heretofore been available to remove inorganic ash and sulfur; however, traditional cleaning has not been able to remove the organic nitrogen and organic sulfur compounds which, upon combustion, produce the SO<sub>x</sub> and NO<sub>x</sub> pollutants. Heretofore precombustion technologies such as fluidized bed boilers, which require limestone as an SO<sub>x</sub> reactant, and post-combustion technologies such as scrubbers or NO<sub>x</sub> selective catalytic convertors have been the main focus in seeking to alleviate these pollution problems. These

devices clean the combustion and flue gas rather than the fuel and are tremendously expensive from both capital and operating standpoints, adding to the cost of power. This added power cost not only increases the cost of domestically produced goods, but also ultimately diminishing this nation's competitiveness with foreign goods. Moreover, operation of post-combustion pollution control equipment draws on the power generated in the plant, reducing saleable plant output. This inefficiency results in higher production of CO<sub>2</sub> per unit of power available for sale. CO<sub>2</sub> production has been linked with the "greenhouse" effect, i.e. the warming of the earth's atmosphere.

It would, therefore, be advantageous to clean up the coal by removing the organic nitrogen (fuel nitrogen) as well as both the organic and the pyritic sulfur while providing a uniform, highly reactive fuel which burns at a lower temperature, thereby reducing the production of thermal NO<sub>x</sub>.

In order to overcome some of the inherent problems with coal as a solid fuel, various methods have been proposed for utilizing coal to produce synthetic liquid or gaseous fuels. These liquefaction or "synfuel" processes are capital intensive and require a great deal of externally supplied water and hydrogen, i.e., hydrogen and water provided from other than the coal feedstock. These processes are also energy intensive in that most carbon atoms in the coal matrix are converted to hydrocarbons, i.e., no pure carbon. This differs markedly from merely "rearranging" existing hydrogen in the coal molecule as in hydrodisproportionation, to hydrogenate certain carbon atoms at the expense of other carbon atoms.

Coal pyrolysis is a well-known process whereby coal is thermally volatilized by heating the coal out of contact with air. Different pyrolysis products may be produced by varying the conditions of temperature, pressure, atmosphere, and/or material feed. Traditional pyrolysis has produced very heavy hydrocarbon tars and carbon (char), with the liberation of hydrogen.

In prior art pyrolysis, as shown in FIG. 2, the pulverized coal is heated relatively slowly at low heating rates and long residence times such that the coal molecule undergoes a decomposition at reaction rate 'k<sub>1</sub>' to yield "decomposition" products, primarily free radical hydrocarbon fragments. These "decomposition" products undergo a recombination or "condensation" reaction at reaction rate 'k<sub>2</sub>', producing char and dehydrogenated hydrocarbons and liberating hydrogen. The decomposition reaction is not desirable in a refining process because it liberates valuable hydrogen instead of utilizing it to upgrade the hydrocarbon products. As shown in FIG. 2, when k<sub>1</sub> and k<sub>2</sub> overlap, the dehydrogenation of the decomposition product, i.e., condensation reaction, is predominant. It is believed that when the coal is heated slowly, the decomposition reaction takes place within the coal particle where there is little hydrogen present to effect the hydrogenation reaction. Thus, the decomposed molecular fragments condense, which results in the production of heavy tar-like liquids of very limited utility.

Other prior art processes for treatment of bituminous and subbituminous coals of various ranks attempted to hydrogenate decomposition products by adding external hydrogen. These hydropyrolysis processes have been carried out in both the liquid and gaseous phases with the most economical processes taking place under milder conditions. However, these processes have had

only limited success in producing economical products. As in pyrolysis, if the heating rates are not rapid, the decomposition material remains inside the coal particles and cannot be hydrogenated by external hydrogen. In order to promote hydrogenation, more stringent reaction conditions were employed, reducing the economic viability. Examples of such processes are disclosed in U.S. Pat. Nos. 4,704,134; 4,702,747; and 4,475,924. In such processes, coal is heated in the presence of hydrogen or a hydrogen donating material to produce a carbonaceous component called char and various hydrocarbon-containing oil and gas components. Many hydropyrolysis processes employ externally generated additional hydrogen which substantially increases the processing cost and effectively makes the process a "liquefaction" process.

A particular type of coal hydropyrolysis, flash hydropyrolysis, is characterized by a very short reactor residence time of the coal. Short residence time (SRT) processes are advantageous in that the capital costs are reduced because the feedstock throughput is so high. In SRT processes, high quality heat is required to effect the transformation of coal to char, liquids and gases.

In many processes, hydrogen is oxidized within the reactor to gain the high quality heat. However, the oxidation of hydrogen in the reactor not only creates water but also reduces the amount of hydrogen available to hydrogenate hydrocarbons to produce higher quality fuels. Thus, in prior art processes, either external hydrogen is required or the product is degraded because valuable hydrogen is converted to water.

The prior art methods of deriving hydrogen for hydropyrolysis are either by: (1) purchasing or generating external hydrogen, which is very expensive; (2) steam-methane reforming followed by shift conversion and CO<sub>2</sub> removal as disclosed in a paper by J. J. Potter of Union Carbide; or (3) char gasification with oxygen and steam followed by shift conversion and CO<sub>2</sub> removal as disclosed in a paper by William J. Peterson of Cities Service Research and Development Company.

All three of these hydrogen production methods are expensive, and a high temperature heat source, such as direct O<sub>2</sub> injection into the hydropyrolysis reactor, is still required to heat and devolatilize the coal. In the prior art processes, either carbon (char) is gasified by partial oxidation, such as in a Texaco gasifier (U.S. Pat. No. 4,491,456 to Schlinger and U.S. Pat. No. 4,490,156 to Marion et al.), or oxygen is injected directly into the reactor. One such system is disclosed in U.S. Pat. No. 4,415,431 (1983) of Matyas et al. When oxygen is injected directly into the reactor, it preferentially combines with hydrogen to form heat and water. Although this reactor gives high-quality heat, it uses up hydrogen which is then unavailable to upgrade the hydrocarbons. This also produces water that has to be removed from the reactor product stream and/or floods the reactor. Additionally, the slate of hydrocarbon co-products is limited.

Flash hydropyrolysis has additional drawbacks in that the higher heating rates associated with short residence times tend to thermally hydrocrack and gasify the material. This gasification reduces liquid yield and available hydrogen.

Thus, it would be advantageous to have a means for producing: (1) a high yield of liquid hydrocarbons, (2) high quality heat for volatilization, (3) hydrogen, and (4) other reducing gases prior to the reaction zone with-

out producing large quantities of water and without using up valuable hydrogen.

In U.S. Pat. Nos. 4,671,800 and 4,658,936, it is disclosed that coal can be subjected to pyrolysis or hydropyrolysis under certain conditions to produce a particulate char, gas and a liquid organic fraction. The liquid organic fraction is rich in hydrocarbons, is combustible, can be beneficiated and can serve as a liquid phase for a carbonaceous fluidic fuel system. The co-product distribution, for example hydrocarbon fractions such as BTX and naphtha, and the viscosity, pumpability and stability of the fuel when the char is admixed with the liquid organic fraction are a function of process and reaction parameters. The rheology of the fuel system is a function of solids loading, sizing, surfactants, additives, and oil viscosity.

The economic feasibility of producing the fluidic fuel is predicated on the method of volatilizing the coal to produce the slurry and a slate of value-added co-products. The economics of transporting the fluidic fuel is predicated upon the rheology of the fuel system.

Common volatilization reactors include the fluidized bed reactor which uses a vertical upward flow of reactant gases at a sufficient velocity to overcome the gravitational forces on the carbonaceous particles, thereby causing suspension of the particles in a gaseous medium. The fluidized bed reactor is characterized by particles subjected to longer reaction residence times to obtain conversion into liquid and gaseous hydrocarbons. Thus, this type of reactor is not very conducive to short residence time (SRT) processing and may produce a large quantity of polymerized (tar-like) hydrocarbon co-products.

Another common reactor is the entrained flow reactor which utilizes a high-velocity stream of reactant gases to impinge upon and carry the carbonaceous particles through the reactor vessel. Entrained flow reactors are characterized by smaller volumes of particles and shorter exposure times to the high-temperature gases. Thus, these reactors are useful for SRT-type systems.

In one prior art two-stage entrained flow reactor, a first stage is used to react carbonaceous char with a gaseous stream of oxygen and steam to produce hydrogen, oxides of carbon, and water. These products continue into the second stage where volatile-containing carbonaceous material is fed into the stream. The carbonaceous feed reacts with the first-stage gas stream to produce liquid and gaseous hydrocarbons, including large amounts of methane gas and char.

Prior art two-stage processes for the gasification of coal to produce primarily gaseous hydrocarbons include U.S. Pat. Nos. 4,278,445 to Stickler; 4,278,446 to Von Rosenberg, Jr.; and 3,844,733 to Donath. U.S. Pat. No. 4,415,431 issued to Matyas et al. shows use of char as a carbonaceous material to be mixed with oxygen and steam in a first-stage gasification zone to produce a synthesis gas. Synthesis gas, along with additional carbonaceous material, is then reacted in a second-stage hydropyrolysis zone wherein the additional carbonaceous material is coal to be hydropyrolyzed.

U.S. Pat. No. 3,960,700 to Rosen describes a process for exposing coal to high heat for short periods of time to maximize the production of desirable hydrocarbons.

One method of terminating the volatilization reaction is by quenching the products either directly with a liquid or gas, or by use of a mechanical heat exchanger. In some cases, product gases or product oil are used.

Many reactors, including those for gasification have employed a quench to terminate the volatilization reaction and prevent polymerizing of unsaturated hydrocarbons and/or gasification of hydrocarbon products. Some have employed intricate mechanical heat-exchange quenches to attempt to capture the heat of reaction. One such quench scheme is shown in U.S. Pat. No. 4,597,776 issued to Ullman et al. The problem with these quench schemes is that they introduce mechanical apparatus into the reaction zone. This can cause tar and char accumulation on the heat-exchanger devices, thereby fouling the heat exchanger.

Thus, if the coal has a hydrogen-to-carbon ratio of 1, and if the hydrogens on half the carbons could be transferred or "rearranged" to the other half of the carbons, then the result would be half the carbons with 0 hydrogens and half with 2 hydrogens. The first portion of carbons (with 0 hydrogens) is char; the second portion of carbons (with 2 hydrogens) is a liquid product similar to a petroleum fuel oil. If this could be accomplished using only hydrogen inherent in the coal, i.e., no external hydrogen source, then the coal could be refined in the same economical manner as petroleum, yielding a slate of refined hydrocarbon products and char.

It would be highly advantageous to have a fuel system which is easily and efficiently prepared solely from coal using no external water and producing a slate of clean burning co-products including benzene, toluene, xylene (BTX); ammonia; sulfur; naphtha; fuel oil; and methanol as well as a clean burning boiler fuel which is: (1) transportable using existing pipeline, tanker car and tankship systems; (2) burnable either directly as a substitute for oil in existing oil-fired combustion systems with little or no equipment modification, or separable at the destination to provide a liquid hydrocarbon fuel or feedstock and a burnable char; (3) a uniform product regardless of the region from which the coal is obtained; (4) high in BTU content per unit weight and volume; (5) high in solid loading and stability; (6) low in ash, sulfur and nitrogen; and (7) free of other polluting effluents which would have to be disposed of at the production site or at the destination.

Further, it would be highly advantageous to have a system for refining coal wherein short residence times and internally generated hydrogen are used in mild conditions in the presence of a catalyst to efficiently produce larger quantities of hydrocarbon liquids without excess gasification of such products. In such a system, inherent hydrogen in the coal could be conserved to increase the co-product value and minimize the process operating costs.

In U.S. patent application Ser. No. 277,603, now U.S. Pat. No. 4,938,782 issued Jul. 3, 1990, it is disclosed that coal can be refined in the presence of internally generated hydrogen to effect high oil yields, without attendant gas production and heavy tar formation. It has now been unexpectedly discovered that the production of hydrocarbon liquids can be greatly increased by use of a catalyst which is introduced into the reactor with the feedstock and/or contained on a medium within the reactor. Surprisingly, the carbon conversion of the coal feedstock and the hydrocarbon liquids is greatly increased by use of a catalyst.

#### SUMMARY OF THE INVENTION

The instant invention relates to an improved method for refining coal by catalyzed short residence time hy-

drodisproportionation to produce a fluidic fuel system and a slate of valuable co-products.

It has now been unexpectedly discovered that catalyzed short residence time hydrodisproportionation (SRT-HDP) processes can be carried out at lower pressures and higher volatilization temperatures to effect higher carbon conversion and increased liquid yields without attendant gas production and/or "condensation" reactions by the presence in the reaction zone of certain catalysts which are preferably fed with the coal feedstock.

In accordance with the invention, particles of volatile-containing carbonaceous material are coated or admixed with a catalyst and heated with hot hydrogen-rich gas at a rate effective to rapidly decompose and volatilize the solid, organic material. The addition of the catalyst promotes "cracking" or depolymerization of the heterocyclic ring compounds which comprise a portion of the solid organic material, thereby increasing the quantity of decomposed and volatilized material to effect a high carbon conversion and an increased liquid yield. The decomposition reaction volatilizes the solid organic material into hydrocarbon fragments and free radicals, causing them to "exit" the carbonaceous particle. These volatilized, hydrocarbon fragments are intimately contacted with a hydrogen donor in a hydrogen-rich gaseous reducing atmosphere in the presence of the catalyst material at a hydrogenation temperature effective to promote the "hydrogenation" of the fragments and free radical "hydrogen capping" and to inhibit condensation. Although some hydrocracking occurs (depending upon the hydrogenation temperature), the catalyst, the hydrogenation temperature, and the hydrogenation residence time are selected to reduce thermal hydrocracking and gasification. By rapidly heating the particles of carbonaceous material to a volatilization temperature effective to decompose the solid organic material and then hydrogenating the decomposition product at hydrogenation temperatures, stable, high quality hydrocarbon liquids are produced from internally generated hydrogen while minimizing gas production from both the "condensation" reaction and hydrocracking. Thus, depolymerization and high heating rates can be obtained to increase the decomposition reaction rate while hydrogenation temperatures are selected to effect efficient hydrogenation of decomposition products, without promoting attendant gasification and/or decomposition reactions.

The present process involves an improved catalyzed method for refining a volatile containing carbonaceous material to produce a slate of hydrocarbon-containing products by short residence time hydrodisproportionation. The process contemplates a heating step wherein volatile-containing carbonaceous particles are rapidly heated in the presence of a catalyst at a rate effective to minimize condensation and the formation of char to volatilization temperatures effective to depolymerize and produce decomposed and volatilized product. The decomposed product is contacted with a hydrogen donor-rich gaseous atmosphere at a hydrogenation temperature to effect hydrogenation and hydrogen capping of the decomposed, volatilized material. The hydrogenation is accomplished at residence times effective to complete hydrogenation of the fragments. It is believed, without limiting the invention, that the presence of the catalyst, in addition to promoting depolymerization of the carbonaceous material, promotes hydrogenation of the volatilized material. The hydrogenated material can

then be quenched to a stabilization temperature below the reaction temperature to prevent deterioration of the liquid products to gas by thermal hydrocracking and/or to inhibit the condensation reaction.

5 In a preferred embodiment, the solid carbonaceous particles are coated with a catalyst, preferably an ion based catalyst, by deposition of said catalyst on the solid carbonaceous particles to provide a uniform catalyst loading. The heating rate in the heating step is such that the decomposition reaction rate is optimized. Contacting the volatilized material with a hydrogen donor-rich gas in a reducing atmosphere is carried out at conditions such that said decomposed volatiles are hydrogenated to maximize oil yield.

15 In a preferred embodiment, the hydrogen donor-rich gaseous reducing atmosphere is obtained in substantial part from the carbonaceous material. In one embodiment, the hydrogen donor-rich gas and/or hydrogen is present in the HDP mixing gas. In another embodiment, the hydrogen donor-rich gas is used as a first quench stream to reduce the temperature below the decomposition temperature and to effect a hydrogenation temperature. In accordance with a further preferred embodiment, the hydrogenated material is quenched further to effect stabilization, i.e., prevent further hydrocracking and/or condensation reaction of the liquids.

20 In another embodiment, the hydrocarbon-containing decomposition vapor from the hydrodisproportionation reaction is subjected to an initial partial quench to hydrogenation temperatures in a hydrogen donor-rich gaseous reducing atmosphere by contacting said vapor with a heavy oil component (primarily hydrocarbons boiling above about 700° F.) recovered from the HDP vapor and recycled. This initial quench, in addition to reducing the temperature of the decomposition vapor, increases the temperature of the heavy oil to a sufficiently high temperature to effect a "thermal cracking" of the heavy oil to lighter oil. Preferably, a second quench medium, which can comprise water and light oil (primarily hydrocarbons boiling below about 400° F.) recovered from the HDP vapor, is used to reduce the temperature of the vapor to effect stabilization. In a greatly preferred embodiment, a partial oxidation reactor is used to produce the heat for volatilization/decomposition and to generate the hydrogen donor-rich gaseous atmosphere.

#### BRIEF DESCRIPTION OF THE DRAWINGS

FIG. 1 is a flow sheet schematic for the catalyzed coal hydrodisproportionation ("HDP") process of the present invention where numbered blocks refer to unit process steps and/or facilities as contemplated by the practice of the instant invention and described in the following specification.

FIG. 2 is a depiction of the reaction rates and reactions associated with the prior art pyrolysis as well as those associated with the HDP reactions of the present invention.

#### DESCRIPTION OF THE PREFERRED EMBODIMENT

The process of the instant invention commences with coal feedstock received at the plant battery limits. Referring to FIG. 1, the feedstock is conveyed to coal and catalyst preparation unit 10 where the coal is reduced to size and partially dried, if necessary. The hot, sized and partially dried coal is directly contacted with an aqueous catalyst solution or slurry, such as  $\text{FeSO}_4$ ,  $\text{FeCl}_2$ ,

and  $\text{Fe}_2\text{O}_3$ , in a spray dryer where the water is evaporated, leaving the catalyst deposited on the coal particles. The coal, coated with catalyst, is then separated from the vapor, pressurized, and sent to hydrodisproportionation and quench unit 16. Steam, recycled gas from gas separation unit 22, and oxygen from the air separation plant (not shown) are reacted as first stage reactions in partial oxidation (POX) unit 14 to produce a hydrogen-rich reducing gas at a high temperature (as later more fully described). The hot POX gas provides the heat, hydrogen, and reducing atmosphere (CO) necessary for short residence time hydrodisproportionation (SRT-HDP) of the carbonaceous material in the hydrodisproportionation and quench unit 16 as well as the make-up hydrogen needed for hydrotreating the HDP liquids in the downstream hydrotreating and fractionation unit 34.

In an SRT-HDP reactor and quench unit 16, the coal coated with catalyst from unit 10 is contacted with the hot POX gas from unit 14 and by hot recycled hydrogen from gas separation unit 22. The coal coated with catalyst is rapidly depolymerized and hydrodisproportionated to HDP vapors and a lesser amount of char. The residence time in the reactor is from about 2 milliseconds to about 100 milliseconds and preferably 10 milliseconds to 75 milliseconds and more preferably 15 milliseconds to 50 milliseconds, depending on the rank of the coal and the reactivity of the catalyst. In order to prevent cracking and continued reactions (polymerization and/or condensation) of heavy, unsaturated hydrocarbons, the HDP vapor is initially quenched to a hydrogenation temperature in the order of from about 900° F. to about 1500° F., and preferably from about 1000° F. to about 1300° F. in the lower portion of the SRT-HDP reactor with recycle liquid, preferably in an initial or upstream quench of heavy oil. Subsequently, the hydrogenated materials are stabilized by a secondary or down stream quench to stabilization temperatures below 1000° F., and preferably below 900° F. by a light oil/water mixture quench. The catalytically promoted hydrogenation reaction occurs for residence times well known in the art depending upon temperature. Residence times of from about 0.1 to about 5.0 seconds are sufficient.

The char produced in unit 16 is separated from the HDP vapors in the char and catalyst separation unit 18 and sent to cooling and beneficiation unit 20. The cooled char is beneficiated by, for example, electrostatic precipitation to remove ash and catalyst particles. In slurry preparation unit 36, the beneficiated char is mixed with hydrotreated oil, methanol and an emulsifying amount of water to produce a non-polluting fluidic fuel system which is a co-product of the instant invention. The refuse from char beneficiation, containing primarily carbon, ash, and spent catalyst, can be combusted in a fluidized bed boiler which comprises the char refuse combustion unit 12 to produce steam required in the POX unit 14. The water to produce the steam is obtained from the water treatment unit 28.

The hot quenched HDP vapors are cooled to recover heat and scrubbed to remove residual char dust in cooling and separation unit 24. The condensed oil and water are separated. The separated oil is sent to hydrotreating and fractionating unit 34.

The separated water is stripped in water treating unit 28 to remove dissolved gases and ammonia. Anhydrous ammonia is then recovered as a co-product and sent to storage (not shown). The stripped water is concentrated

in unit 28 where dissolved organics and salts are concentrated in a small fraction of the water. The concentrate, which is high in hydrocarbon content, is then moved to slurry preparation unit 36 for use as emulsifying water in the preparation of the fluidic fuel system. The distillate water from the concentrator is used to produce steam in the char refuse combustion unit 12. Thus, there is no water discharge effluent from the facility.

The non-condensed cooled sour gas from unit 24, which has been scrubbed to remove char dust, is conveyed to the gas purification unit 32 where sulfur compounds, trace impurities and most of the carbon dioxide are removed. Naphtha range hydrocarbons in the gas are also removed in unit 32 and moved to hydrotreating and fractionating unit 34. The removed sulfur components are sent to a sulfur recovery unit 26 where the sulfur is recovered by conventional means as a co-product and sent to storage (not shown). The separated  $\text{CO}_2$  from unit 32 is compressed by conventional means to about 2,000 psia and removed by pipeline (not shown) as a co-product for use in enhanced oil recovery, agriculture, and the food industry.

The purified gas from gas purification unit 32 is sent to a "once-through" methanol synthesis unit 30 where, in a single pass, part of the  $\text{H}_2$ ,  $\text{CO}$  and  $\text{CO}_2$  in the gas is converted by the catalytic converter to methanol and water. The crude methanol produced is purified in unit 30 by, for example, distillation, and pure methanol is separated and moved to storage (not shown). A high concentration of methanol in a water stream (up to 95% methanol by volume) is also separated and moved to the slurry preparation unit 36 for preparation of the fluidic fuel system. This stream negates the necessity for expensive methanol purification while providing a diluent and thermal  $\text{NO}_x$  suppressant to the fluidic fuel. Unreacted gases are purged from the methanol synthesis unit and moved to gas separation unit 22.

In gas separation unit 22, the purged gas from methanol synthesis is separated into two streams; a hydrogen rich gas and a methane/carbon monoxide-rich gas. Part of the separated hydrogen-rich gas is compressed and heated prior to recycle to the SRT-HDP reactor in unit 16. The remainder of the hydrogen-rich gas is sent to hydrotreating and fractionation unit 34. The methane/carbon monoxide rich gas is heated and then recycled to the partial oxidation unit 14.

The naphtha range hydrocarbons from unit 32 are hydrotreated and benzene-toluene-xylene (BTX) is then separated by extractive distillation in unit 34. The BTX and naphtha are removed to storage (not shown). The separated oil (380° F. + boiling hydrocarbons) from unit 24 is also hydrotreated in unit 34. Part of the hydrotreated oil is moved to unit 36 to be mixed with char to produce the instant fluidic fuel and the remainder of the hydrotreated oil is sent to storage (not shown) as a low sulfur fuel oil co-product. This hydrotreated oil has a heating value in excess of 18,000 Btu/lb and is substantially devoid of  $\text{SO}_x$  and  $\text{NO}_x$  producing compounds.

#### Feedstock

The carbonaceous materials that can be employed as feedstock in the instant process are, generally, any volatile-containing material which will undergo hydrolytic destructive distillation to form a particulate char and volatilization products. Bituminous and subbituminous coals of various ranks as well as waste coals and lignites are examples. Peat may also be used.

Anthracite, which contains minimal volatiles, is not a preferred feedstock.

Preferably, coals from the lignite rank to the medium volatile bituminous rank are used. Lignites are an advantageous starting material for the instant invention since they contain process water for hydrodisproportionation and manufacture of methanol, as well as up to 55% by weight volatiles (on a dry basis). Additionally, combining the coal with a catalyst, as disclosed herein, increases liquid yield and lowers the viscosity of such liquids. The mining and preparation is fully described in Kirk-Othmer ENCYCLOPEDIA OF CHEMICAL TECHNOLOGY, second edition, Vol. 5, pp. 606-676. The coal is mined by either strip or underground methods as appropriate and well known in the art.

The raw coal, which preferably has a particle size of less than about 5 cm, is normally subjected to crushing to reduce the particle size. Preferably, the coal is pulverized to 70 percent minus 200 mesh. The need for size reduction and the size of the reduced material depends upon the process conditions to be used, i.e., the heating rate and the volatilization temperature, as well as the composition and rank of the coal material, particularly its agglomerating tendencies and the inorganic sulfur and ash content of the coal. When beneficiation is necessary, for example, with coals containing a high percentage of ash or inorganic sulfur, the coal is preferably ground and subjected to washing and beneficiation techniques. When coals are used which have agglomerating tendencies, the size of the coal must be matched to the hydrodisproportionation techniques and process conditions in order to produce a particulate char and to prevent agglomeration during HDP.

#### Feedstock Preparation

Referring to FIG. 1, unit 10 includes coal receiving, storage, reclaiming, conveying, grinding, drying, and catalyst deposition facilities required to prepare the coal for introduction to the HDP unit 16. This unit 10 also includes facilities to grind or pulverize the feed coal from a received size of 5 cm to 70 percent minus 200 mesh and to dry the coal to from about 1% to 12% by weight moisture and preferably 2% to about 4% by weight moisture.

The crushing, pulverizing and/or grinding can be accomplished with any equipment known in the art, but preferably is accomplished with impact mills such as counter-rotating cage mills, hammer mills or the like. The pulverizers are swept with a stream of heated gas which partially dries the coal. Pulverizer outlet temperature is maintained at from about 250° to about 500° F. and preferably from 300° F. to about 400° F.

The pulverized coal is pneumatically conveyed to a spray dryer where it is contacted with an aqueous catalyst solution or slurry. The water is evaporated by contact with the hot coal particles, resulting in the catalyst being deposited on the coal particles. Catalyst-to-coal weight ratios of from about 0.025 to about 0.15 are required. In another embodiment, a dry catalyst, preferably  $\text{Fe}_2\text{O}_3$ , is mixed with the pulverized coal downstream of the pulverizer to produce a uniform coal-catalyst mixture. The coal coated with catalyst and/or the catalyst/coal mixture is separated from the gas in cyclone separators. Part of the gas from these cyclones is returned to the pulverizer circuits and the remainder of the gas is sent to a bag house prior to being vented to the atmosphere. Fugitive dust collectors are provided at transfer points to minimize coal dust emissions to the

atmosphere. Advantageously, carbonaceous fines and the like are subjected directly to hydrodisproportionation. The catalyst coated coal from the cyclone separators and bag filter is sent to a coal feed surge bin. The coal is normally fed through lockhoppers which are pressurized with high pressure nitrogen from the air separation plant. After an upper lockhopper is filled with coal, it is then pressurized prior to its discharging coal to the lower lockhopper. The emptied upper coal lockhopper is then depressurized to atmospheric pressure and is again filled with coal from the surge bin. Lockhopper valves are controlled, for example, by a microprocessor unit which is used to control the coal filling, pressurization, coal feeding, and depressurization sequence.

#### Partial Oxidation

Referring to FIG. 1, the POX process, depicted as unit 14, may comprise any pressurized partial oxidation reactor capable of producing synthesis gas ( $\text{H}_2$  and  $\text{CO}$ ). This process produces hydrogen, high quality heat and a reducing atmosphere ( $\text{CO}$ ) for the hydrodisproportionation reaction, as well as the production of hydrogen for downstream hydrotreating and for reducing sulfur and nitrogen. The POX process may be combined as a first stage of the HDP reactor or, preferably, may be accomplished in a separate unit as shown in FIG. 1. In the POX reactor, methane/carbon monoxide-rich gas and steam are sub-stoichiometrically reacted with oxygen to produce a hydrogen-rich gas,  $\text{CO}$ , and high quality heat. The  $\text{CH}_4/\text{CO}$ -rich gas is preferably reaction gas from the gas separation unit 22 discussed hereinbelow. The hydrogen-rich gas, the  $\text{CO}$  and unreacted steam from the POX reactor are at a high temperature and provide the required heat and reducing atmosphere necessary for hydrodisproportionating the coal.

More specifically, in the present process, a fuel gas, preferably a  $\text{CO}$ -rich methane, and more preferably a purified reaction gas, is introduced into a first-stage reactor with oxygen. The oxygen is present in an amount less than the stoichiometric amount required to react with all of the fuel gas. An amount of steam sufficient to preferentially inhibit the production of water is also introduced. The steam is preferably derived from preconditioning the coal. The  $\text{CO}$  in the gas stream is preferred for the selective production of hydrogen by extraction of an oxygen from water. This occurs in accordance with one or more of the following reactions:



Generally, the oxygen is introduced into the first-stage reactor in an amount to provide a molar ratio of oxygen to  $\text{CH}_4/\text{CO}$  within a range from about 0.3 to about 1.25 and preferably from about 0.40 to about 0.90, and more preferably from about 0.5 to about 0.75 based on a methane-to-CO volumetric ratio of 1 to 1. These ratios will change depending upon the requirement for the heat generated and the composition of the exit gas, specifically the required partial pressure of  $\text{H}_2$ .

The oxygen, fuel gas and steam are reacted in the first-stage POX reactor at a pressure of from about 100 psig to about 1,200 psig, and preferably from about 400 psig to about 800 psig, and more preferably from about 500 psig to about 700 psig; and at a temperature within the range from about 1,300° F. to 3,000° F., and preferably from about 1,500° F. to 2,500° F., and more preferably from about 1,800° F. to about 2,300° F.

The first-stage reaction produces a hot gas stream principally comprising hydrogen, CO and steam along with carbon dioxide and minor amounts of other gases such as nitrogen or the like. The temperature within the stage-one reaction is controlled such that the hot gas stream produced is essentially free (for example, totaling less than 0.1 volume percent of the total gas stream) of hydrocarbons, oxygen moieties and hydroxymoieties, although there can be a small amount of methane, depending on the conditions. The hot gas stream is preferably mixed with recycle hydrogen from the gas separation unit 22 (described hereinbelow) which has been heated to about 1,000° F. The resulting gaseous mixture having a uniform temperature is then injected into the HDP reactor.

#### Hydrodisproportionation and Quench

Coal and catalyst (either as a catalyst deposited on the pulverized coal or as an admixture of coal and catalyst) from coal and catalyst preparation unit 10 is fed to the hydrodisproportionation (SRT-HDP) reactor and quench unit 16 by gravity and differential pressure. The coal and catalyst is preferably injected into the reactor through a central feed nozzle where the coal, in the presence of the catalyst, is rapidly heated to effect depolymerization and disproportionation at a thermal equilibrium mix temperature of from about 1,000° F. to about 2,000° F., and preferably at about 1,500° F. to 1,750° F. for bituminous coals and 1,300° F. to 1,500° F. for sub-bituminous and lignites. The admixed catalyst promotes depolymerization of the coal molecules and significantly increases the yield to liquid hydrocarbons. The coal is heated by contact with hot, hydrogen-containing gas.

As discussed hereinabove, in the POX process substoichiometric oxygen and steam are contacted with reaction gas (CH<sub>4</sub>/CO rich), preferably from gas separation unit 22, to obtain products including primarily CO, H<sub>2</sub> and heat. This hot gas is contacted in the SRT-HDP reactor with coal and catalyst from unit 10 to rapidly heat the coal to volatilization temperatures. Recycled hydrogen from the gas separation unit that has been preheated to about 1,000° F. can be simultaneously fed to the reactor. Preferably, the coal is heated by intermixing with the gas to from about 1,000° F. to about 2,000° F. at from about 100 psig to about 1,200 psig and is hydrodisproportionated with the volatilized material undergoing hydrogenation.

The hot POX gas rapidly heats the coal at a rate of at least about 10,000° F./second and at ranges from about 10,000° F./second to about 250,000° F./second.

Prior to contacting the coal, the hot gas is accelerated to a velocity to effect intimate contact of the particulate coal with the hot gas stream and to volatilize the coal within a residence time in the reactor of from about 2 milliseconds to about 100 milliseconds, and preferably from about 10 milliseconds to about 75 milliseconds, and more preferably from about 15 milliseconds to about 50 milliseconds, depending on the rank of the coal. Prior to contacting the coal, the hot gas is accelerated

ated to a velocity of from about 200 feet per second to about 1,000 feet per second, and preferably from about 300 feet per second to 800 feet per second, and most preferably from about 400 feet per second to 600 feet per second to effect mixing of solid and gas.

The amount of particulate coal and the amount of hot gas introduced into the HDP reactor can be controlled to produce the desired reaction temperature and residence time. The higher the partial pressure of hydrogen, CO, and steam in the HDP reactor, the more saturated hydrocarbons and CO<sub>2</sub> are produced. The reactants and products from the HDP process are rapidly cooled to effect the desired total hydrodisproportionation reaction exposure time.

The prior art injected oxygen into the second stage reaction for heat. Any oxygen present in the second stage reaction of the instant invention is from oxygen in the coal molecule. The important aspect is that there is no "free" oxygen in the feed to the HDP reactor so that water formation is not the preferential reaction.

The first- and second-stage processes may be accomplished in two separate reactors or within a single vessel. In this latter configuration, the carbonaceous feed is introduced into the hot gas from the first stage to effect the second stage. The direction of flow of the products through the reactors or vessel is dependent only upon the longitudinal axial alignment of the reactors or single reactor vessel. The direction of product movement through the first and second stages is not limited to either upflow or downflow when a high velocity propelling force is used to overcome gravitational forces and to insure proper heating profiles and rapid product movement through the reactors. Thus, by using high velocity flows to propel the reaction products through the reactors, the direction of axial alignment of the reactors or vessel can be varied.

Preferably, the first stage of the process is accomplished in a separate unit. In this method, the outlet end of a POX reactor section is connected in close proximity to the inlet end of a reaction section designed to accomplish the second-stage reaction. The two reactor sections can comprise two physically separate, compatible reactors utilizing a high product flow rate, short-residence time, entrained-flow reactor; or the two reaction stages may be integral parts or zones of a single unit. The direction of axial alignment of the reactor is not important since high velocity entrained flow is not gravity dependent so long as the high rate of flow and short exposure time required to achieve the desired product slate is provided.

This two-stage process can be used for the hydrodisproportionation of any solid or semi-solid or even liquid carbonaceous material. Preferably, oxygen is introduced to the POX unit 14 in substoichiometric amounts to maintain the desired operating temperature range in the second-stage volatilization. Steam is added to effect material balance, to enhance the phase shift reaction, and to inhibit the production of water. The amounts are empirical to the feedstock and desired product slate. Steam requirements are therefore dependent upon the second-stage carbonaceous material feed rate, the type of carbonaceous feed introduced, and the operating conditions in the second stage, etc.

Higher temperatures and longer high temperature exposure times in the second stage create a need for greater amounts of hydrogen in the second stage as heavy hydrocarbons are cracked to lighter material. In order to meet second-stage hydrogen requirements, for

example, 0.05 to 0.25 pounds of  $H_2$  per 1 pound of carbonaceous material is required to be fed into the second stage.

The instant process, which involves the rearranging of hydrogen and the use of hydrogen from constituents in the carbonaceous material, has certain limits. Specifically, the amount of hydrogen that can be produced in this manner is finite. It has been found, however, that with most coals other than anthracite, devolatilization of the coal, cracking of heavier material, and even hydrogenation of some portion of the solid carbon is possible. Of course, the more hydrogen in the feedstock, the more valuable is the fuel produced.

A refractory-lined reactor vessel can be used to volatilize the carbonaceous material. This vessel can be a single vessel for the combined stage-one and stage-two processes, or for the stage-two process only. The refractory lined second-stage vessel can be cylindrical or rectangular in shape.

As part of the second-stage reactor configuration, an injector system is preferably used for rapidly injecting the particulate coal and catalyst and rapidly admixing and heating the coal and catalyst with a hot, hydrogen-rich stream of reducing gases. The coal injector can be centrally located or can comprise a series of manifolded injectors dispersed on the head portion of the reactor. The carbonaceous material and hot gas are preferably injected through rectangular shaped slots with the hot gas stream injection angle not greater than 60 degrees when measured from a horizontal plane. The means for particle injection can be any means known in the art such as gravitational flow, differential pressure, entrained flow, or the like.

FIG. 2 shows the distinction between the hydrodisproportionation reaction of the instant invention and the prior art pyrolysis process. The following is advanced as explanatory theory only and should not be construed as a limitation of the instant invention. The rapid volatilization and decomposition of volatile containing carbonaceous material is accomplished by heating the carbonaceous material very rapidly to effect a high heating rate (second order function) to a volatilization temperature. This heating rate has been found to increase  $k_1$  and minimize the "condensation" reaction rate  $k_2$  (see FIG. 2). When decomposition is accomplished at higher heating rates, i.e., in excess of 10,000° F., the decomposed volatilized material is "blown out" of the particle as low molecular weight hydrocarbons which contain free radical sites. If hydrogen is present in the atmosphere surrounding this decomposed material as it exits the particle, the decomposed material is hydrogenated. If the condensation reaction is allowed to proceed at lower heating rates, then the presence of hydrogen in the atmosphere is not as effective.

However, in order to effect high heating rates, the mixing temperature must be relatively high to impart sufficient energy to the coal particle to heat it rapidly in milliseconds of time. These high temperatures, however, militarily affect the formation of hydrogenated liquids and promote cracking to gaseous products which use up hydrogen and degrade liquid production.

By immediately adjusting the temperature of the decomposed volatilized material to a hydrogenation temperature (as opposed to stopping the reaction by "stabilization quenching") in the presence of hydrogen,  $k_3$  is increased such that hydrogenated, light liquids are produced. As is seen in the reaction schemat in FIG. 2, the concentration of decomposition material available

to undergo the "condensation" reaction with reaction constant  $k_2$  is minimized. It is also theorized, without limiting the scope of the invention, that the catalyst reduces the activation energy, allowing hydrogenation to occur at lower temperatures and effectively inhibiting the condensation reaction to increase overall carbon conversion. This results in increased liquid yields as well as improved stability and quality of the liquid products. Adjustment of temperature to a hydrogenation temperature in the presence of the catalyst also minimizes high temperature thermocracking to gases heretofore believed a necessary product of high heating rate volatilization processes.

The hydrogenated products may be further quenched to cease all reactions after the decomposition products have been sufficiently hydrogenated. Thus, in accordance with the instant invention, the initial heating rate of the coal does not have to determine the ultimate slate of volatilization products, including large amounts of gas, and the condensation reaction can be effectively avoided.

Anterior of the reactor vessel, disposed in an annular fashion about the circumference of the vessel, are one or more sets of quench nozzles through which a quench medium is dispensed to slow down and/or terminate the reaction and to reduce the temperature of the reaction products.

#### Hydrogenation

The hydrogenation is preferably accomplished by reducing the reactant temperature to inhibit excessive hydrocracking and promote catalytic hydrogenation. Temperatures in the range of from about 900° F. to about 1500° F., and preferably in the range of from about 1100° F. to about 1300° F. are sufficient at residence times in the order of from about 0.1 seconds to about 5.0 seconds. The temperature reduction is preferably accomplished in a single or series of quench steps. Hydrogen rich gas is a preferred quench medium. Heavy process oils which undergo hydrocracking during the quench are greatly preferred.

#### Quench

The HDP vapor is subjected to an instant quench to stop the volatilization reaction and provide a direct heat exchange. This may take place in two or more steps which may be overlapping. In a particularly preferred embodiment, a two-step quench is used to minimize the condensation reaction, i.e., formation of high viscosity tars and/or the formation of gas. In the first step, the heavy oil (primarily hydrocarbons boiling about 700° F.) produced in the HDP reaction is recycled as a primary quench medium. This medium is injected directly through a first set of quench nozzles into a reactor chamber to effect a temperature reduction to hydrogenation temperatures, as well as a "thermal cracking" of the heavy oil and tars.

The second quench step (if used) preferably uses recycle water and lighter oils (primarily hydrocarbons boiling at less than 400° F.) to reduce the temperature of the HDP volatiles to a stabilization temperature below about 900° F., preferably from about 700° F. to about 900° F., to prevent reaction (polymerization) of unsaturated hydrocarbons and free radicals and to inhibit further "thermal cracking" to gas.

In this quench process, there are no indirect heat exchangers and the heat for the fractional distillation is transferred to the liquids to be distilled directly by inter-

action in the reactor in this quench step. Thus, no re-heating is required and a "step down" process is provided. This also allows further generation of lighter oils for slurring the char and precludes the need to use the tars for an enhanced solid product.

The quantity of quench liquid is determined by its latent heat of vaporization and heat capacity or ability to absorb the sensible heat of the HDP vapors. The quench liquid can comprise any liquids or gases that can be blended rapidly and in sufficient quantity with the reactant mixture to readily cool the mixture below the effective reaction temperature. The cooling down or quenching of the reactant HDP vapors can occur within the HDP reactor or subsequent to the departure of the gases from the HDP reactor. For example, the reactant vapors can be quenched in the pipe line between the HDP reactor and char separator by quench nozzles located in the pipe line.

The short exposure time in the HDP is conducive to the formation of aromatic liquids and light oils. It has been found that rapid heating and catalyzed depolymerization of carbonaceous materials not only "drives out" the volatiles from the feed particles (devolatilization), but also thermally cracks larger hydrocarbons into smaller volatiles which escape from the host particle so rapidly that condensate reactions are largely bypassed. With a rapid quench to hydrogenation temperatures, these volatiles are stabilized first by reaction with hydrogen to form a less reactive product and then by lowering the internal energy of the volatiles below the reactive energy level. The net result is the rapid production of these volatiles to prevent polymerization to heavy oil or tar (high molecular weight compounds) and the maximization of lighter hydrocarbon liquids.

#### Reactor Products

The HDP reactor product slate includes primarily H<sub>2</sub>, CO, CO<sub>2</sub>, H<sub>2</sub>S, NH<sub>3</sub>, H<sub>2</sub>O, C<sub>1</sub> to C<sub>4</sub> hydrocarbons, benzene, toluene, and xylene, minus 700° F. boiling liquids and plus 700° F. boiling liquids. The product slate is dependent upon the coal type and operating parameters, such as pressure, temperature, and second-stage residence time, which can be varied within the reactor system. It has been found that the presence of CO, CO<sub>2</sub>, and CH<sub>4</sub> in the feed to the second-stage HDP reactor does not inhibit the production of benzene, toluene, xylene (BTX) and other liquid products in a short-exposure time, high-temperature hydropyrolysis. CH<sub>4</sub> and CO<sub>2</sub> are merely diluents which have little effect on the second-stage reactions. The concurrent presence of water vapor is required to inhibit the formation of water (H<sub>2</sub> +  $\frac{1}{2}$  O<sub>2</sub> → H<sub>2</sub>O) and the net reaction extracts hydrogen from water to provide some of the hydrogen consumed in the hydrogenation reactions. Hydrogen is extracted from water vapor in the first stage to satisfy the hydrogen needs in the second-stage.

The total carbon conversion, expressed as the percentage of the carbon in the gases and liquids found in the second-stage end products to the total amount of carbon in the second-stage carbonaceous feed material, ranges from about 50 weight percent to about 80 weight percent. The component carbon conversion expressed as the percentage of carbon converted to that component in the second-stage end product to the amount of carbon in the second-stage carbonaceous feed material ranges as follows: C<sub>1</sub>-C<sub>4</sub> hydrocarbons from about 5 weight percent to about 25 weight percent; BTX from about 5 weight percent to about 25 weight percent;

minus 700° F. boiling liquids (excluding BTX) from about 20 weight percent to about 40 weight percent; and plus 700° F. boiling liquids from about 10 weight percent to about 30 weight percent.

The second-stage product gases are useful for the extraction of marketable by-products such as ammonia, a hydrogen source for hydrotreating the product oil, a fuel for use in combustion systems, and a feedstock for the production of lower chain alcohols which can be used as a hydrocarbon-rich liquid to alter the viscosity of the slurry liquids and the flow characteristics of the slurry. In accordance with a preferred embodiment, these gases are used primarily to produce lower chain alcohols which are admixed with the liquid organic fraction. Advantageously, the gases are "sweetened" prior to being marketed or used in the process. The elimination of potential pollutants in this manner not only enhances the value of the slurry as a non-polluting fuel but also improves the economics of the process since the gaseous products may be captured and marketed or utilized in the process.

#### Char Separation

The quenched HDP vapor and char is sent to a primary char separator, unit 18 in FIG. 1, where the catalyst and most of the char are separated from the vapor. The vapor stream is then sent to a secondary separator to remove additional char. The vapor, now containing only a small amount of char dust, is conveyed to cooling and separation unit 24.

The separated char and spent catalyst can then be fed to a lockhopper system for depressurization to atmospheric pressure. Solid material discharged from the lockhoppers is normally fed to surge bins. The char from these storage bins can then be pneumatically conveyed with nitrogen to char cooling and beneficiation unit 20.

#### Char Cooling and Beneficiation

Particulate char is preferably fed to facilities, unit in FIG. 1, for cooling and beneficiation prior to mixing it with hydrotreated oil from hydrotreating and fractionation unit 34 to produce a fluidic fuel system. This char is normally cooled from about 900° F. to about 100° F.

The hot char is cooled to about 520° F. by generating 600 psig steam in a series of heat exchangers also for use in the partial oxidation unit 14. The char is further cooled to 100° F. to 145° F. by cooling water in a second set of heat exchangers. The cooled char is sent to a separator where the char is separated from the carrier gas (nitrogen) before going to storage bins. (Nitrogen, a surplus by-product of oxygen manufacture, is an inert carrier gas). The cooled char is fed to an electrostatic precipitator where ash and catalyst particles are separated from the carbonaceous char particles. In the electrostatic precipitator, from about 70 percent to about 90 percent of the char heating value is recovered in the beneficiated char stream and the remainder is contained in the char ash and catalyst refuse stream. The beneficiated char, containing less than 10% by weight ash and catalyst constituents, is sent to fluidic fuel preparation unit 36. The refuse from char beneficiation is sent to a boiler, for example, a fluidized bed boiler unit 12, to generate the steam required in partial oxidation unit 14.

#### Fluidic Fuel System Preparation

The beneficiated char, part of the hydrotreated oil, methanol and water are preferably mixed to produce a

substantially combustible fluidic fuel. Preferably, this fuel is a three-phase system comprising solid char, hydrocarbons and an amount of water effective to form an emulsion. Cooled, beneficiated char from char cooling and beneficiation unit 20 is fed to a char storage bin. The char is fed through a feeder to a mix tank where the char is mixed with hydrotreated oil from hydrotreating and fractionation unit 34, hydrocarbon-rich condensed water from the condenser in unit 28, and a methanol/water mixture from methanol synthesis unit 30. The fluidic fuel product from the mix tank is then pumped to storage (not shown).

#### Cooling and Separation (Fractional Condensation)

The char dust is scrubbed from the HDP vapor and the HDP is cooled and condensed. The facilities to accomplish this processing are represented in unit 24 of FIG. 1. Cooling and separation unit 24 accepts HDP vapor having a temperature of from about 700° F. to about 1,000° F. and preferably at about 850° F. in four consecutive cooling steps. Liquid hydrocarbons and water are also condensed and collected for separation in an oil-water separator. Facilities are also available to scrub ammonia to less than 10 ppm in the gas before being sent to gas purification unit 32.

In a first cooling step, HDP vapor at about 850° F. from char separation unit 18 is cooled to about 520° F. in a heat exchanger where saturated steam is generated. The partially cooled HDP vapor stream is sent to a scrubber and then to a vapor-liquid separator where condensed heavy hydrocarbons are separated from the cooled vapor stream. Part of the condensed liquid from the bottom of the separator is recirculated to the scrubber where it contacts the HDP vapor stream to remove residual entrained char dust from the HDP vapor. The remainder of the condensed heavy oil is recycled to the HDP reactor and quench unit 16 as the primary quench fluid.

In a second cooling step, the HDP vapor at about 520° F. is circulated through a second heat exchanger where it is cooled to about 300° F. by generating lower temperature saturated steam. This cooled stream is moved to a second separator where condensed oil and water are separated from the vapor in an oil-water separator in unit 24.

Vapor from this second separator is circulated through a third heat exchanger in a third cooling step where it is further cooled to about 290° F. by preheating boiler feed water. The liquid-vapor stream then goes to a third separator for separation of the liquid from the vapor. The separated liquid stream (oil and water) is sent to an oil-water separator.

In a fourth cooling step, vapor from the third separator is sent to an air cooler where it is cooled to about 145° F. with air and then cooled to about 100° F. by a water cooled exchanger.

The cooled vapor-liquid stream goes to a fourth separator (bottom section of the ammonia scrubber) where the light condensed oil and water are separated. The vapor then goes to a packed bed section in the ammonia scrubber where it is contacted with water to remove any remaining ammonia and acid gas. Part of the condensed oil and water from the bottom of the ammonia scrubber is used as the final quench liquid for the hot HDP vapor produced in the SRT-HDP reactor. The remainder of the condensed light oil and water is sent to an oil-water separator within the cooling and separation unit 24.

The oil-water separator in unit 24 is designed to separate the condensed oil from water in the three oil/water streams and to provide intermediate storage of the separated oil and water streams.

5 The heavy oil-water stream from the second separation is cooled and sent to a heavy-oil expansion drum where the pressure is reduced and where most of the dissolved gases in the heavy-oil water mixture are released. The degassed heavy oil-water mixture is sent to 10 a heavy oil separator where heavy oil is separated from lighter oil and water. The lighter oil and water are then sent to another oil-water separator where the light oil is separated from the water. The separated heavy oil and light oils are then sent to oil run-down tanks. Water from the bottom of the separator is sent to a sour water storage tank.

15 The medium oil-water stream from the third separator is cooled, then mixed with the light oil-water stream from the fourth separator and sent to a medium and light oil expansion drum. The released gas is mixed with the gas from the heavy oil expansion drum and then cooled to about 100° F. in a water cooled heat exchanger. The oil-water mixture from the expansion drum is sent to a separator where the oil is separated 20 from the water. Separated oil is sent to an oil run-down tank from which it is pumped to the hydrotreating and fractionation unit 34. Water from the bottom of this oil separator is also sent to the sour water tank before being sent to unit 28 water treating.

25 Sour ammonia-containing water is sent to an ammonia still (steam stripper) where acid gas and ammonia are stripped from the water and anhydrous ammonia with a purity of greater than 99.5 wt. percent is recovered. Stripped water from the bottom of the ammonia still is sent to flash drum where a small amount of the water is flashed and recycled to the still. Remaining water from the flash drum is separated into two streams. One stream goes to a water cooled exchanger where the stripped water is cooled for re-use in the plant as previously described. The second stream is sent to a brine concentrator where dissolved organics and salts are concentrated in a brine stream. The concentrate is sent to slurry fuel system preparation unit 36. A useful water treatment/ammonia stripping and recovery section is 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880

covered along with a naphtha product, both of which are useful as gasoline blending stock and/or chemical feedstock.

The oil hydrotreating section hydrotreats and stabilizes the oil such that it will not polymerize, and desulfurizes the oil to less than 0.15 percent sulfur. The oil hydrotreater also reduces nitrogen to less than 2000 ppm and oxygen to less than 100 ppm. This process renders the fluidic fuel produced from this oil substantially free of fuel NO<sub>x</sub> and SO<sub>x</sub> pollutants in accordance with one aspect of the instant invention.

In a preferred embodiment, a process is employed for further treating the liquid organic fraction to adjust viscosity. Numerous processes for hydrotreating liquid hydrocarbons are known and readily available in the art. The paramount consideration in the present invention is to obtain a maximum amount of liquids having a viscosity consistent with producing a fluidic fuel that is capable of pipeline transport and of loading a maximum of a particulate solid coal char while being combustible in a liquid-fueled combustion system.

The separated liquid hydrocarbons ("oil") require further treatment to increase the hydrogen-to-carbon ratio and to reduce the sulfur and nitrogen content. This is accomplished by contacting the oil with hydrogen in a catalytic reactor ("hydrotreater") at moderate pressure and temperature. The hydrogen reacts with the sulfur and nitrogen contained in the oil to produce hydrogen sulfide and ammonia and further hydrogenates the oil. Light oil is separated from heavier oil and then further processed to separate benzene, toluene, and xylene (BTX), and naphtha.

#### Gas Purification

All of the gas handling facilities required for gas purification are represented by unit 32 in FIG. 1. Sour gas from the cooling and separation unit 24 is sent to gas purification where sulfur components are removed to less than 0.2 ppm and carbon dioxide is reduced to about 3.0 percent so the resultant gas may be used in the methanol synthesis unit 30. Naphtha range hydrocarbons, and trace quantities of ammonia and hydrogen cyanide are also removed from the gas. An example of such a commercially available gas purification unit is the "Rec-tisol" process licensed by Lurgi, Frankfurt, West Germany.

A compressor for carbon dioxide is included in unit 32. CO<sub>2</sub> off-gas separated from the sour gas in gas purification unit 32 is sent, for example, to a two case, electric motor driven, centrifugal compressor where the CO<sub>2</sub> is compressed in 4 stages with air coolers followed by water cooled exchangers. An air after-cooler followed by a water cooler is also provided to cool the compressed (fluid) CO<sub>2</sub> to about 100° F. prior to being sent to a pipeline.

Sour gas from cooling and separation unit 24 is cooled by cool purified gas and refrigerant to condense residual water vapor in the gas. The condensed water is separated from the gas and sent to water treating unit 28.

The cooled gas is then sent to an H<sub>2</sub>S absorber. The gas is contacted with a solvent in the bottom of the H<sub>2</sub>S absorber to remove naphtha boiling range hydrocarbons plus residual water, ammonia, and hydrogen cyanides. The gas then flows to the main H<sub>2</sub>S absorber section where H<sub>2</sub>S and COS are removed by cold CO<sub>2</sub>-laden solvent.

The desulfurized gas then goes to a CO<sub>2</sub> absorber where most of the CO<sub>2</sub> is removed from the gas by cold regenerated solvent. The cold, purified gas is heated by cross-exchange with the incoming sour gas prior to being sent to methanol synthesis and purification unit 30.

The solvent containing H<sub>2</sub>S, COS and CO<sub>2</sub> from the H<sub>2</sub>S absorber is flashed to release dissolved gases (H<sub>2</sub>, CO, CH<sub>4</sub>, etc.). The solvent is further depressurized in a series of flashes to remove part of the dissolved CO<sub>2</sub>. The enriched H<sub>2</sub>S solvent stream is sent to hot regeneration.

CO<sub>2</sub>-rich solvent from the CO<sub>2</sub> absorber is flashed to release dissolved gases and is then further flashed to remove part of the dissolved CO<sub>2</sub>. The partially regenerated solvent is recycled to the mid-section of the CO<sub>2</sub> absorber.

The released CO<sub>2</sub> from the CO<sub>2</sub> flash tower and from the H<sub>2</sub>S reabsorber are combined, heated and sent to the CO<sub>2</sub> compressor and then to a CO<sub>2</sub> pipeline. H<sub>2</sub>S-rich solvent from the H<sub>2</sub>S reabsorber is heated by cross exchange with hot regenerated solvent from the regenerator and then stripped in the hot regenerator to separate dissolved H<sub>2</sub>S, COS, CO<sub>2</sub> and light hydrocarbons.

25 The stripped gas is sent to sulfur recovery unit 26.

The solvent stream from the bottom of the H<sub>2</sub>S absorber containing naphtha and dissolved gases is flashed in a pre-wash flash tower. The flashed gases are recycled to the H<sub>2</sub>S re-absorber. The solvent-naphtha stream from the flash tower is sent to a naphtha extractor where the naphtha is separated from the solvent. The recovered raw naphtha is sent to hydrotreating and fractionation unit 34. The water-solvent stream from the extractor is sent to an azeotrope column. Residual

35 naphtha, dissolved gases and some water and solvent are stripped in the overhead of the azeotrope column and recycled to the pre-wash flash tower. Water-solvent mixture from the bottom of the azeotrope column is pumped to the solvent-water column where the solvent is stripped from the water and sent to the regenerator. Waste water from the bottom of the solvent-water column is collected and sent to water treating unit 28.

#### Sulfur Recovery

45 Sulfur from the various sour gas streams produced in the plant is recovered by facilities represented as unit 26. Acid gas from gas purification unit 32 is sent to an H<sub>2</sub>S absorber where hydrogen sulfide and some of the carbon dioxide in the gas is absorbed using, for example, 50 a SCOT solvent. The desulfurized gas, containing primarily light hydrocarbons, hydrogen and carbon dioxide are sent to the plant fuel gas header. The solvent from the absorber containing hydrogen sulfide and carbon dioxide is sent to a solvent stripper where the H<sub>2</sub>S and CO<sub>2</sub> are stripped from the solvent. The stripped acid gas is then sent to a reaction furnace. The H<sub>2</sub>S is converted to elemental sulfur by methods well known in the art. An example of such a device is a Claus unit. The sulfur produced is sent to a sulfur storage unit (not shown).

#### Once-Through Methanol Synthesis and Purification

65 In accordance with one aspect of the instant invention, crude methanol is produced in a once-through reactor and part of the crude methanol is purified to meet Federal Grade AA specifications. This area, represented by unit 30 of FIG. 1, also produces a methanol-rich water stream for mixing with the fluidic fuel to

enhance rheological properties and reduce thermal NO<sub>x</sub> emissions. The remainder of the methanol is used as an oxygenated motor fuel.

Purified gas from gas purification unit 32 is compressed to methanol synthesis pressure in, for example, a turbine driven synthesis gas compressor. Part of the compressed gas is cooled in, for example, a water cooled exchanger and sent to gas separation unit 22. The remainder of the gas is heated by cross exchange with the methanol reactor effluent gas and fed to the methanol reactor. In the reactor, part of the hydrogen reacts with carbon monoxide to produce methanol and a minor amount of hydrogen reacts with carbon dioxide to produce methanol and water. Only about 20% of the hydrogen fed to the methanol reactor is actually converted to methanol. The hydrogen is internally produced as set forth hereinbefore. Small amounts of organics and other alcohols are also produced in the reactor. The preferred reactor is an isothermal catalytic reactor in which the gas flows through tubes containing a catalyst. The exothermic heat of reaction is removed by transferring heat to boiler feed water on the outside of the tubes and generating medium pressure steam.

The effluent gas and methanol from the reactor is partially cooled by preheating the feed gas to the reactor. The stream is further cooled by an air cooler and then a water cooler to condense the contained methanol and water. The non-condensable gas, primarily hydrogen, carbon monoxide and methane with lesser amounts of carbon dioxide, ethane and nitrogen, is purged from the system and sent to unit 22 gas separation. In this process, there is no requirement to compress and recycle the purified gas to the methanol synthesis reactor. This eliminates the expensive compression and recycle steps required in typical methanol processes and allows methanol to be produced as an economical co-product of the present process.

The condensed crude methanol, containing water, dissolved gases, and trace amounts of produced organics, is sent to a pressure let-down drum where part of the dissolved gases and light organics are released. The crude methanol is then sent to a stripper column where the remaining dissolved gases and light organics are stripped. The stripped crude methanol is then sent to a distillation column where pure methanol is recovered in the overhead, condensed and sent to storage. In a conventional process, essentially all of the methanol must be separated, making the process energy intensive and expensive. In the instant process, only part of the methanol is separated, with the remaining methanol-rich water portion from the bottom of the distillation column being sent to fluidic fuel preparation unit 36.

#### Gas Separation

Hydrogen is separated from purified HDP gases, which are primarily CH<sub>4</sub>/CO (purge gas) in gas separation facilities represented by unit 22 of FIG. 1. The hydrogen is recompressed and heated prior to its recycle to the hydrodisproportionation and quench unit 16. In addition, part of the separated hydrogen is sent to 60 hydrotreating and fractionation unit 34 for use in naphtha production and oil hydrotreating. Most of the separated gas, primarily methane and carbon monoxide, is heated and sent to the partial oxidation unit 14.

Purge gas from once-through methanol synthesis unit 30 is sent to a scrubber where any residual entrained solvent is removed by methods well known in the art. The solvent should be removed from the gas to prevent

fouling of the membrane separator in gas separation unit 22. Gas from the scrubber is heated prior to going to the membrane separators. In the membrane separator, H<sub>2</sub> is separated from the other gases by semipermeable membranes formed, for example, into hollow fibers. The separated hydrogen (containing small amounts of CO<sub>2</sub>, CO, and CH<sub>4</sub>) is compressed in a hydrogen compressor. Part of the compressed, hydrogen rich gas is sent to a heater where the hydrogen rich gas is heated and then recycled to hydrodisproportionation and quench unit 16. The remainder of the hydrogen rich gas is sent to hydrotreating and fractionation unit 34. The separated gas consisting primarily of methane and carbon monoxide is heated and sent to the partial oxidation unit 14.

#### Fluidic Fuel

The terms "fluidic fuel" or "liquid/solid mixture" as used herein are meant to include a composition having an amount of the particulate coal char which is in excess of that amount which is inherently present in the liquid organic portion as a result of the hydropyrolysis process.

For most applications, the particulate coal char constituent should comprise not less than about 45% by weight of the composition and preferably from about 45% to about 75% by weight. In accordance with one aspect wherein the char is separated from the liquid at the fuel system destination, the term 'fluidic fuel' is intended to include a composition containing amounts of char as low as 1% by weight, which composition may be further transported, for example, by pipeline, to a refinery or to another combustion facility.

If the fluidic fuel is to be fired directly into a liquid fueled combustion device, the loading and the liquid organic constituents and the viscosity of the liquids may be varied to maximize combustion efficiency, and, in some cases, amounts of alcohol and "make up" hydrocarbon distillates can be added. This enhances combustion characteristics in a particular combustion system configuration and reduces thermal NO<sub>x</sub> while enhancing rheology characteristics of the slurry.

Liquid petroleum distillates which can be used include fractions from petroleum crudes or any artificially produced or naturally occurring hydrocarbon compound which is compatible with the coal-derived liquid organic hydrocarbon containing portion used as the fluidic medium in accordance with the instant invention. These would include, without limitation, the aliphatic, cyclo-aliphatic and aromatic hydrocarbons, heterocyclics and phenols as well as multi-ring compounds, aliphatic-substituted aromatics and hydroxyl-containing aliphatic-substituted aromatics. The term aliphatics is used herein to include both saturated and unsaturated compounds and their stereo-isomers. It is particularly preferred to add the lower chain alcohols, including the mono-, di- and trihydroxyl compounds. Preferably, the make-up hydrocarbons do not contain mercaptan, sulfate, sulfite, nitrate, nitrite or ammonia groups.

Preferably, the chars are discrete spherical particles which typically have a reaction constant of from about 0.08 to about 1.0, a reactivity of from about 10 to about 12; surface areas of from about 100 microns to about 200 microns; pore diameters of from about 0.02 milimicrons to about 0.07 milimicrons; and pass 100 mesh, and preferably 200 mesh. Similar chars are described in U.S. Pat. No. 4,702,747. The useful chars have a high reactivity and surface area, providing excellent Btu to weight

ratios. They are finely divided particles as distinguished from the larger, "structured" particles of the prior art. The char particles are sufficiently porous to facilitate beneficiation and combustion but the pore size is not so large as to require the use of excessive liquid for a given amount of solid.

It is important, in order to obtain the requisite liquid/solid mixture having the desired rheological characteristics, that the solid component be discrete, particulate char. The spherical shape of the char particles allows adjacent particles to "roll over" one another, thereby improving slurry rheology and enhancing the solid loading characteristics. When utilizing agglomerating or "caking" coals, preferably the process parameters are regulated so as not to produce an agglomerated char product.

Except for coal feedstocks with an exceptionally low ash content, the char produced during the process should be beneficiated prior to being admixed with the process oil. When indicated, beneficiation may be utilized to clean either the coal or the char. The beneficiation can be performed by any device or process known in the art utilized to extract pollutants and other undesirable inorganics such as sulfur and ash. Beneficiation may be accomplished, for example, by washing, jiggling, extraction, oil agglomeration (for coal only), and/or electrostatic separation. The latter three methods remove both ash and pyritic (inorganic) sulfur. When the solvent extraction or oil agglomeration methods are used, it is most advantageous to use the liquid derived from the hydrolysis process as the beneficiating agent. The exact method employed will depend largely on the coal utilized in forming the char, the conditions of hydrolysis, and the char size and porosity.

The char material is ground to yield the substantially spherical, properly sized particulate coal char. Any conventional crushing and grinding means, wet or dry, may be employed. This would include ball grinders, roll grinders, rod mills, pebble mills, and the like. Advantageously, the particles are sized and recycled to produce a desired distribution. The char particles are of sufficient fineness to pass a 100 mesh screen (Tyler Standard) and about 32% of the particles pass a 325 mesh screen. In accordance with the instant invention, char particles in the 100 mesh range or less are preferable. It will be realized that the particulate char of the instant invention having particle sizes in the above range is important to assure not only that the solid is high in reactivity, but also that the fluidic fuel is stable and can be pumped directly into combustion systems.

The exact distribution of particle sizes is somewhat empirical in nature and depends upon the characteristics of the liquid organic fraction. The rheological characteristics of the fluidic fuel are interdependent upon the viscosity of the liquid fraction and the particle size distribution of the char.

The ground, beneficiated char can be sized by any apparatus known in the art for separating particles of a size on the order of 100 mesh or less. Economically, screens or sieves are utilized; however, cyclone separators or the like can also be employed. The spheroid shape of the primary particle provides spacing or voids between adjacent particles which can be filled by a distribution of second or third finer particle sizes to provide bimodal or trimodal packing. This modal packing technique allows addition of other solid fuel material such as coal to the fluidic fuel without affecting the very advantageous rheology characteristics of the par-

ticulate coal char/liquid organic fraction fluidic fuel system of the instant invention. Additionally, this packing mode allows the compaction of substantially more fuel in a given volume of fuel mixture while still retaining good fluidity.

Particulate char produced from certain ranks of coal has pore sizes and absorption characteristics such as to require treating of the char prior to admixing of the particulate char with the liquid to reduce absorption by the char of the liquid phase. Prevention of excessive absorption of organic and/or hydrocarbon liquid by the char is necessary to prevent instability of rheology characteristics. When absorption rates by the char are in excess of from about 10% to about 15%, pretreatment is very beneficial. In accordance with this pretreatment, the char is brought into intimate contact with an amount of the coating or "sealing" material effective to reduce the absorption of liquid by the char. The treatment is effected prior to the particulate char being admixed with the liquid. The sealants or coatings that are useful include organic and inorganic materials which will not produce pollutants upon combustion nor cause polymerization of the fluidic fuel. Since surfactants and emulsifiers are used to enhance fuel stability, care must be taken that the coating or sealant is compatible with the stabilized composition. Sealants and coating materials which are particularly advantageous include paraffins and waxes, as well as the longer chain aliphatics, aromatics, polycyclic aromatics, aro-aliphatics and the like. Mixtures of various hydrocarbons, such as No. 6 fuel oil, are particularly desirable because of their ready availability and ease of application. Advantageously, the higher boiling liquid organic fractions from the hydrolysis of the coal are utilized. The sealant or coating can be applied to the char by spraying, electrostatic deposition or the like. In this manner, one can economically enhance the rheological stability of the fluidic fuel while preserving its usefulness as a non-polluting combustion fuel.

Coal and water, or more preferably the hydrolysis gases, can be used to produce methanol and other lower chain alcohols, preferably in accordance with the method previously described. These alcohols are utilized as a component of the liquid phase for the combustible fuel admixture to adjust liquid viscosity and enhance rheology characteristics.

As used herein the term alcohol is employed to mean alcohols (mono-, di- and trihydroxyl) which contain from 1 to about 4 carbon atoms. These include, for example, methanol, ethanol, propanol, butanol and the like. The alcohol may range from substantially pure methanol to various mixtures of alcohols as are produced by the catalyzed reaction of gases from HDP or natural gas. Advantageously, the alcohol constituent can be produced on site at the mine in conjunction with the HDP reaction.

The admixing of the solid particles with the liquid phase can be accomplished by any well-known mixing apparatus in which an organic liquid constituent and a particulate coal char can be mixed together in specific proportion and pumped to a storage tank. Advantageously, emulsifying techniques are used, such as high speed impellers and the like. The method of admixing, and especially emulsifying, will vary the rheology characteristics of the fluidic fuel. Unlike coal/water slurries and coal/oil mixtures, the fuel of the instant invention is transportable by oil pipeline and does not require mixing equipment at the end-use facility. Thus, even small

process heat systems can utilize the fuel of the instant invention efficiently and economically.

The important rheological aspect of the fluidic fuel in the instant application is that it is pumpable and stable. This is accomplished by matching the size of the solid char particle, the viscosity of the liquid phase and the stabilizer. Preferably, a small percentage by weight, for example from 1% to about 12%, of water is admixed into the fuel system. This is especially preferable when surfactants which have hydrophylic moieties are used. The fuel is preferably agitated or blended to produce a suspensoid which is stable under shear stress, such as pumping through a pipeline.

As discussed above, surfactants, suspension agents, organic constituents and the like may be added depending on the particular application. Certain well-known surfactants and stabilizers may be added depending on the viscosity and non-settling characteristics desired. Examples of such substances which are useful in accordance with the instant invention include dry-milled corn flour, gelatinized corn flour, modified cornstarch, cornstarch, modified waxy maize, guar gum, modified guar, polyvinyl carboxylic acid salts, xanthan gum, hydroxyethyl cellulose, carboxymethyl cellulose, polyvinyl alcohol and polyacrylamide. As hereinbefore mentioned, advantageously the admixture of the instant invention demonstrates high fluidity. Thus a high Btu per unit volume mixture is obtained with lower viscosities and higher fluidities. Certain of the well-known stabilizers create adverse rheological characteristics.

As previously set forth, the sizing and packing of the solid is particularly important in obtaining a highly loaded, stable, transportable combustion fuel system. It has been found advantageous to have the solid material smaller than about 100 mesh (Tyler) and about 32% passing a mesh size in the range of 325. Preferably, the viscosity of the liquid organic fraction is in the range of from 17° API to about 20° API. This will, of course, depend on the loading and pumping characteristics desired, the stabilizers used, and whether coal and/or alcohol are present in the slurry in accordance with the instant invention. The degree API is very important in the end-use application, i.e., the combustion system design. Those oil fired systems designed for "heavier" crudes will tolerate more viscous oils and higher loaded slurries.

#### Catalysts

Several types of catalysts can be used in accordance with the instant invention. The catalysts can be zinc, potassium, sodium, calcium, or iron based; however, since the catalyst is fed with the feedstock in a once-through arrangement, low cost iron based catalysts are greatly preferred. Oxides, sulfates, chlorides, fluorides, nitrates, and other iron salts can be used. Those that are highly soluble in water are preferred. Iron chloride ( $FeCl_3$ ) and iron sulfate ( $FeSO_4$ ) are the greatly preferred catalysts.

#### Pollution Control

As previously stated, the fluidic fuel of the instant invention provides precombustion elimination of pollution causing materials, specifically those which produce  $SO_x$  and  $NO_x$  upon combustion. The coal and/or the char may be beneficiated to remove pyritic sulfur. Organic fuel nitrogen and organic fuel sulfur are removed during the HDP reaction and further in the hydrotreating and fractionation unit 34.

Methanol can be added to the fluidic fuel as previously described in order to reduce the combustion (thermal)  $NO_x$  by reducing the combustion temperature of the slurry. This, along with the uniformity of the fuel and the reactivity of char, greatly reduces the amount of thermal  $NO_x$  as compared with the combustion of raw coal which burns with hot spots.

A pulverized or powdered limestone can be added directly to the fluidic fuel highly in excess of stoichiometric amounts to act as a reactant in the combustion of the fuel to reduce the  $SO_x$  emissions from pyritic sulfur.

#### EXAMPLE

The following example with reference to FIG. 1 is used to demonstrate the feasibility of the instant invention. The SRT-HDP facility is designed to convert 10,000 tons (moisture, ash free) of coal feed per day to a char/hydrocarbon fluidic fuel (one composition of which is set forth later herein) and co-products. In unit 10, dry pulverized coal which is pneumatically conveyed by inert gas at 350° F. is contacted in a spray dryer by 500 tons per day of iron sulfate catalyst dissolved in a 50 weight percent water solution at about 200° F. The water is evaporated in the spray dryer, leaving the iron oxide deposited on the coal particles. The dried coal covered with catalyst is separated from the inert gas and water vapor and fed to a SRT-HDP reactor, unit 16, and subjected to rapid hydrodisproportionation and quench. Approximately 70,000 pounds per hour of hydrogen preheated to 1,000° F. is recycled to the SRT-HDP reactor. Steam (600 psig, 950° F.) from unit 12 and recycle gas at 750° F. from unit 22 are fed to a POX unit 14 at the rates of 400,000 lbs/hr. and 470,000 lbs/hr., respectively. In the POX reactor, the steam and recycled gas are reacted with about 210,000 lbs/hr. of oxygen (substoichiometrically) to produce a hydrogen-rich reducing gas stream at about 2,300° F. and 525 psig. The hot gas from the POX unit is mixed with the heated recycle hydrogen and directly fed to the SRT-HDP reactor operating at about 500 psig to heat the coal and catalyst in about 30 milliseconds to about 1,300° F., at which temperature the coal is volatilized. The volatilization products are partially quenched with recycled heavy oil from unit 24 to about 1,100° F. and partially hydrogenated. The residence time in the hydrogenation section of the SRT-HDP reactor is about one second. The HDP vapors and char are finally quenched to about 850° F. with about 200,000 lbs/hr. hour of recycled quench water/oil mixture, also from unit 24.

The char and catalyst, at a rate of about 315,000 lbs/hr, are separated from the gas and HDP vapor, depressurized to atmospheric pressure, cooled through a heat exchanger (not shown) and sent to char cooling and beneficiation unit 20. The char is beneficiated in unit 20 to produce about 156,000 lbs/hr of low sulfur, low ash char. The refuse from char beneficiation is combusted in unit 12 to produce about 580,000 lbs/hr of 600 psig, 950° F. steam, of which 400,000 lbs/hr is used in the POX unit and the remaining 140,000 lbs/hr is utilized in steam turbine drive process compressors. The gas and HDP vapor is further processed as shown in FIG. 1 to recover liquid hydrocarbons, purify noncondensable gases, separate hydrogen for recycle to the reactor, and recover gas for recycle to the POX unit 14. Beneficiated char and part of the hydrotreated oil is admixed with a methanol-rich water stream to produce the fluidic fuel in unit 36. The fluidic fuel which is pro-

duced has a higher heating value of about 14,400 Btu/lb, with an ash content of about 4.7 weight percent and a sulfur content of less than 0.09 weight percent. The products which can be produced in this configuration include: 3,400 tons per day (TPD) of the fluidic fuel; 4,150 barrels per day (BPD) of BTX; 3,250 BPD of naphtha; 7,800 BPD of low sulfur fuel oil; 1,400 BPD of methanol; 70 TPD of ammonia; 45 TPD of sulfur; and 75 MMSCFD of CO<sub>2</sub> for enhanced oil recovery. This example illustrates the advantage of the invention which produces hydrogen and heat in a first-stage POX reaction for volatilizing the carbonaceous material in the presence of an iron-based catalyst in a HDP second stage.

While the invention has been explained in relation to its preferred embodiment, it is understood that various modifications thereof will become apparent to those skilled in the art upon reading the specification and the invention is intended to cover such modifications as fall within the scope of the appended claims.

What is claimed is:

1. An improved catalytic method for refining a volatile containing carbonaceous material, which method comprises the steps of:

- (a) heating a particulate, volatile containing carbonaceous material in the presence of a catalyst selected from the group consisting of iron-based, zinc-based, potassium-based, sodium-based, and calcium-based catalysts at a heat rate sufficient to maximize decomposition and minimize formation of char and condensation products to a volatilization temperature effective to produce a substantially decomposed volatilization product; and
- (b) contacting said substantially decomposed volatilization product with a hydrogen donor-rich gaseous atmosphere at a hydrogenation temperature effective to minimize formation of condensation products and reduce thermal cracking for a hydrogenation residence time effective to produce a hydrogenated volatilization product.

2. The method of claim 1 wherein said catalyst is iron-based.

3. The method of claim 1 wherein said catalyst is selected from the group of iron-based catalysts consisting of iron oxides and iron salts.

4. The method of claim 1 comprising the further step of producing a stabilized, hydrogenated product by adjusting the temperature of said hydrogenated volatilization product to a stabilization temperature effective to substantially terminate formation of condensation products and thermal cracking of said hydrogenated volatilization product.

5. The method of claim 1 wherein said heating rate is at least about 10,000° F. per second and said volatilization temperature is from about 1,000° F. to about 2,000° F.

6. The method of claim 1 wherein said hydrogenation temperature is from about 900° F. to about 1,500° F. and said hydrogenation residence time is from about 0.1 seconds to about 5.0 seconds.

7. The method of claim 4 wherein said stabilization temperature is below about 1,000° F.

8. The method of claim 1 wherein said hydrogenation temperature is effected by direct partial quench.

9. The method of claim 8 wherein said direct partial quench is effected by using hydrogen donor-rich gas, or heavy hydrocarbon process liquid which heavy hydro-

carbon process liquid is thermally cracked during said partial quench to produce lighter hydrocarbon liquids.

10. The method of claim 1 wherein said hydrogen donor-rich gaseous atmosphere is obtained in substantial part from said carbonaceous material and wherein said hydrogen donor-rich gaseous atmosphere and said volatilizing temperatures are produced in substantial part in a partial oxidation reaction wherein steam and hydrodisproportionation recycle gas rich in methane and carbon monoxide are reacted with a sub-stoichiometric amount of oxygen.

11. The method of claim 10 wherein said catalyst is selected from the group of iron oxides, iron chlorides, and iron sulfates.

12. The process of claim 1 wherein said carbonaceous material is selected from a group consisting of coals, lignites, low rank and waste coals, peats, and mixtures thereof.

13. An improved method for refining a volatile containing carbonaceous material comprising the steps of:

- (a) heating a particulate, volatile containing carbonaceous material in the presence of an iron-based catalyst by admixing said particulate with a gaseous heating medium at a volatilization temperature of from about 1,000° F. to 2,000° F. and at a decomposing heat rate of at least 10,000° F. per second to produce a substantially decomposed volatilization product;
- (b) contacting said substantially decomposed volatilization product in the presence of said catalyst with a hydrogen donor-rich reducing gaseous atmosphere consisting essentially of hydrogen, steam, and carbon monoxide at a temperature of from about 900° F. to about 1,500° F. and at a hydrogenation residence time of from about 0.1 seconds to about 5.0 seconds to produce a hydrogenated volatilization product, said hydrogen and carbon monoxide being formed in substantial part in a partial oxidation reaction wherein steam and a hydrodisproportionation recycle gas rich in methane and carbon monoxide are reacted with a substoichiometric amount of oxygen; and
- (c) cooling said hydrogenated volatilization product to reduce the temperature of said product to below about 1000° F., said cooling accomplished at a rate to provide a total residence time from the heating of said carbonaceous material to said cooling of said hydrogenated volatilization product of between about 0.02 seconds and about 5.0 seconds.

14. The method of claim 13 wherein said catalyst is selected from the group consisting of iron oxides, iron chlorides, and iron sulfates.

15. The method of claim 13 wherein the temperature of which said contacting step is accomplished by direct partial quench.

16. The method of claim 15 wherein said direct partial quench is effected by using a hydrogen donor-rich gas, or heavy hydrocarbon process liquid which heavy hydrocarbon process liquid is thermally cracked during said partial quench to produce lighter process liquids.

17. The method of claim 13 wherein said hydrogen in said reducing gaseous atmosphere is obtained in substantial part from said carbonaceous material.

18. The process of claim 13 wherein said carbonaceous material is selected from a group consisting of coals, lignites, low rank and waste coals, peats, and mixtures thereof.

19. An improved catalyzed method for refining a volatile containing coal to produce a slate of hydrocarbon containing co-products by short residence time hydrodisproportionation, which method comprises the steps of

- (a) contacting a particulate coal in the presence of a catalyst selected from oxides, sulfates, and chlorides of iron, with a hydrogen donor-rich reducing gaseous mixture having a temperature in the range of about 1,300° F. to about 3,000° F. to heat said particulate coal at a volatilization temperature of from about 1,000° F. and about 2,000° F. at a heating rate greater than about 10,000° F. per second at pressures of from about 100 psig to about 1,200 psig for a time of from about 0.002 seconds to about 0.10 seconds to produce a substantially decomposed volatilization product, wherein said hydrogen donor-rich gaseous reducing gaseous mixture is obtained in substantial part from said coal by a partial oxidation reaction wherein steam and hydrodisproportionation recycle gas rich in methane and carbon monoxide are reacted with a sub-stoichiometric amount of oxygen;
- (b) cooling said substantially decomposed volatilization product in the presence of said catalyst to temperatures from about 900° F. to about 1,500° F. for residence times of from about 0.1 seconds to about 5.0 seconds to produce a hydrogenated volatilization product, wherein said cooling is effected by direct partial quench by using a hydrogen donor-rich gas or a heavy hydrocarbon process liquid, which heavy hydrocarbon process liquid is

thermally cracked during said partial quench to produce lighter process liquids; and

- (c) stabilizing said hydrogenated volatilization product at a temperature of less than about 1,000° F. to produce a stabilized hydrogenated volatilization product wherein said stabilization is accomplished by contacting the hydrogenated volatilization product with a mixture of water and lighter oils, said mixture being recycled from said hydrodisproportionation process.

20. The method of claim 19 wherein said catalyst is deposited on said particulate coal prior to said contacting.

21. The process of claim 19 wherein said contacting is accomplished at a volatilization temperature of from about 1,200° F. to about 1,750° F. and a heating rate greater than about 50,000° F. per second and a residence time of from about 9.002 seconds to about 0.03 seconds.

22. The process of claim 19 wherein said cooling is accomplished at temperatures of from about 1,100° F. to about 1,300° F. and residence time of from about 0.1 to about 2.0 seconds.

23. The process of claim 19 wherein said stabilization step is accomplished at temperatures less than about 900° F.

24. The method of claim 19 wherein said partial oxidation reaction is carried out at temperatures of from about 1,800° F. to about 2,500° F. and pressure of from about 300 psig to about 700 psig with a mole equivalent of oxygen to CH<sub>4</sub>/CO of from about 0.5 to about 0.75.

\* \* \* \* \*